

## UNITED STATES PATENT OFFICE

ERWIN SOHN AND RALPH J. PADDOCK, OF BELLEVUE, PENNSYLVANIA, ASSIGNORS TO  
STANDARD SANITARY MFG. CO., OF PITTSBURGH, PENNSYLVANIA, A CORPORATE  
ATION OF NEW JERSEY

## CHROMIUM PLATING

No Drawing.

Application filed November 5, 1928. Serial No. 317,475.

This invention relates to chromium plating and more particularly to a process of electrodepositing chromium and to an electrolytic bath from which chromium can be satisfactorily deposited.

It is an object of this invention to provide an improved process and electrolytic bath for chromium plating.

It is a further important object of this invention to provide an electrolytic solution for chromium plating which has satisfactory throwing power and efficiency for commercial application and from which chromium can be electrodeposited as a bright and smooth coating.

Other and further important objects of this invention will become apparent from the following description and appended claims.

20 It is generally known that in the chromic acid type of chromium plating solutions, in addition to the chromic acid small quantities of an additional acid or acid radical are necessary to provide for satisfactory deposition. Of the acids or acid radicals commonly used, sulphuric acid has probably found the widest application. The present invention concerns itself with a substitute either in part or in whole for the sulphuric acid.

30 We have now found that hydrofluosilicic acid, its alkali metal salts or, in general, any metallic salt of said acid which is dissolved by a chromic acid solution, can be used to replace sulphuric acid, either in whole or in part. Hydrofluosilicic acid is usually obtained as a solution containing from 28 to 35%  $H_2SiF_6$ . The quantities hereinafter referred to are actual amounts of the acid (100%).

35 In carrying out our process, certain conditions are preferably standarized, as follows:

Using lead anodes and a copper cathode, the temperature of the chromium plating bath is kept at 110° F. and a current density of 100 amperes per square foot used with a voltage varying between 3.2 and 4 volts. It will, of course, be understood that these conditions can be varied depending upon the nature of the work to be plated. However, with these conditions maintained, a plating bath having the following range of ingredi-

ents has been found to give a chromium deposit with good cathode efficiencies:

CrO<sub>3</sub>----- 150 to 450 gr. per liter  
 $H_2SiF_6$ ----- 0.30 to 12.0 gr. per liter

While a plating bath consisting of chromic acid and hydrofluosilicic acid alone will deposit chromium and with good cathode efficiency and throwing power as compared to a solution containing sulphuric acid, the nature of the chromium deposit is not entirely satisfactory. We therefore prefer to use with the hydrofluosilicic acid, small quantities of sulphuric acid within the range of 0.35 to 1.05 gr. per liter, but in this case the quantity of hydrofluosilicic acid to be used is considerably reduced, say not to exceed a maximum of 3 gr. per liter.

Our preferred composition of chromium plating bath is as follows:

CrO<sub>3</sub>----- 208 gr. per liter  
 $H_2SO_4$ ----- 0.35 gr. per liter  
 $H_2SiF_6$ ----- 0.60 gr. per liter

Using our preferred plating solution, a satisfactory cathode efficiency, say of 16%, can be obtained and the chromium plated out is bright and smooth. Furthermore, the throwing power of the solution is very good. Further additions of hydrofluosilicic acid do not greatly affect the efficiency until about 2.6 grams per liter of hydrofluosilicic acid are present in the solution, but the throwing power of the solution decreases with the first addition, at which point 0.60 grams per liter of hydrofluosilicic acid had been added. A solution containing 0.35 grams per liter of sulphuric acid and 0.60 grams per liter of hydrofluosilicic acid is a good working solution, having good throwing power and efficiency.

The fact that the sulphate ion content of the chromium plating bath can be reduced below the equivalent of 1 gr. per liter of  $H_2SO_4$  by replacing a part of the sulphuric acid normally used with hydrofluosilicic acid and excellent plating results obtained, is quite unexpected and probably not in accord with published data on chromium plating.

In place of hydrofluosilicic acid, alkali

metal salts of the acid may be used, such as sodium fluosilicate, or as stated, most any metallic salt which is soluble in a chromic acid solution, for instance, chromium fluosilicate. For calculating the amount of metallic fluosilicate, the equivalent of hydrofluosilicic acid is used within the above range. Likewise, in place of sulphuric acid, introduced as such, metallic salts of sulphuric acid may be used. It will therefore be understood that by the terms sulphuric acid and hydrofluosilicic acid, as used in the claims, is meant either the free acids or salts of said acids capable of furnishing in solution the respective acid radicals.

Due to the fact that commercial chromic acid, in general, contains appreciable quantities of sulphates, it is usually necessary to take special steps to control the sulphate content of a plating solution prepared from commercial chromic acid and hydrofluosilicic acid. A method of control has been described in the copending application of Erwin Sohn, Serial No. 294,940, filed July 23, 1928, which comprises determining the sulphate content of the solution analytically and adding a calculated amount of barium carbonate to precipitate the excess of sulphate ions as barium sulphate. By this method the sulphate content of the solution may be brought down to 0.35 grams per liter of equivalent  $H_2SO_4$  or less. If the sulphate content is brought below the desired amount, sufficient sulphuric acid may be added and then the desired quantity of hydrofluosilicic acid introduced until the solution possesses the desired efficiency and throwing power. It has been found advisable to filter the solution after the precipitation of excess sulphate with barium carbonate.

In contrast with other plating solutions, it has been found that boric acid has no value in a chromium plating solution containing chromic acid and hydrofluosilicic acid. In fact, the effect of boric acid is harmful.

We are aware that numerous details of the process may be varied through a wide range without departing from the principles of this invention, and we, therefore, do not purpose limiting the patent granted hereon otherwise than necessitated by the prior art.

We claim as our invention:

1. The process of chromium plating, which comprises passing an electric current through a bath containing from 150 to 450 grams of chromic acid, from 0.35 to 1.05 grams of sulphuric acid and from 0.30 to 3.0 grams per liter of hydrofluosilicic acid to the article to be plated as cathode.

2. The process of chromium plating, which comprises passing an electric current through a bath containing approximately 200 grams of chromic acid, approximately 0.35 grams of sulphuric acid, and approxi-

mately 0.60 grams of hydrofluosilicic acid per liter of solution to the article to be plated as cathode.

3. A chromium plating bath, consisting of a solution of 150 to 450 grams of chromic acid, 0.35 to 1.05 grams of sulphuric acid and 0.30 to 3.00 grams of hydrofluosilicic acid.

4. A chromium plating bath, consisting of approximately 200 grams of chromic acid, 0.35 grams of sulphuric acid and 0.60 grams of hydrofluosilicic acid per liter of solution.

5. A chromium plating bath of high throwing power, comprising a 15 to 45% solution of chromic acid having a mixed stable acid content of from 0.65 to 4.05 grams per liter of solution, said stable acid content being composed of a relatively strong and a relatively weak inorganic acid, said relatively weak inorganic acid being hydrofluosilicic acid in an amount ranging from 0.6 to 3.0 grams per liter of solution.

In testimony whereof, we have hereunto subscribed our names at Pittsburgh, county of Allegheny, Penna.

ERWIN SOHN.  
RALPH J. PADDOCK.

90

95

100

105

110

115

120

125

130